

## UNITED STATES PATENT OFFICE.

ROBERT A. MARR, OF NORFOLK, VIRGINIA.

## PULP AND FIBER PRODUCT AND PROCESS OF MAKING SAME.

No Drawing.

Application filed February 2, 1923. Serial No. 616,609.

The present invention relates to the production of fiber, pulp, and paper by the use of a particular class of treating liquids which have not heretofore been employed in the manufacturing of pulp from wood or other vegetable materials so far as I have been advised.

In my U. S. patent application No. 407,759, filed September 2, 1920, of which the present case is in part a continuation, I have described and claimed the process of making pulp by treating organic materials containing cellulose, with a digestive solution containing copper sulfate, iron sulfate, or with other sulfates such as those of cobalt, nickel, manganese and chromium, and said application also mentioned the use of double sulphates of certain metals with the sulfates of the alkali metals, and magnesium sulfate is also mentioned therein.

The present invention is in its more specific aspect based upon the use of a soluble sulfate of an alkali-forming metal (i. e., alkali sulfate or magnesium sulfate) as the principal constituent of the digestive solution although it is to be understood that such sulfates can be used in conjunction with other metal-sulphates as will appear below. In its broader aspect, the present case involves the use of a digestive solution including a sulfate of a metal having an atomic weight between 23 and 63.6, such solution being preferably of a concentration of about 0.5 to 5 ounces (preferably below 4 ounces) per gallon, such solution being much more dilute than the digestive solutions heretofore generally employed in this country.

Among the prior processes, it may be noted that there is a so-called "sulphate process", which is a somewhat incorrect name, since in the said "sulphate process" the alkali metal sulfate employed is, before it is used for the digestion of the wood, ordinarily in large part reduced to the corresponding sulfid, and a solution of the sodium sulfid or other alkali metal sulfid, usually also containing considerable free alkali, forms the real digestive solution. In my process, I use no alkali metal sulfid and no free caustic alkali.

In the present process it is possible to successfully employ the solutions of alkali metal sulphate which are very much less concentrated than are the ordinary cooking liquors used in the manufacture of pulp, for example, I find that a strength of from one

to four ounces (preferably about one and one-half ounces to three ounces) of the sulphate per gallon of liquor gives excellent results. Further this liquor, at the end of the cooking operation, after separation from the cooked chips or cooked wood in blocks or other cellulosic material can be put back into the digester and used again with another batch of chips or blocks. The digestive liquor can be used over many times, but it is advisable to add to the liquor from time to time, say after every fourth, or fifth cook, an amount of the sulfate equal to a minor fraction, say about one-fourth of the amount originally employed.

I give the following examples of procedure falling within the scope of the invention, but it is to be understood that these examples are given as illustrative and not as restrictive.

## Example 1.

White birch was cut into chips, averaging about one-half a cubic inch in size. The chips in this particular example were packed in a cage and the cage then placed in the digester, with a solution containing 1.8 ounces per gallon (1.4%) of sodium sulphate alone. An amount of digestive solution equal to about seven gallons of the said solution per ten pounds of wood was added, this being sufficient to completely cover the said chips. The liquor was then heated, until the steam pressure in the digester was about 100 pounds per square inch, which condition was maintained for about 60 minutes. The source of heat was then shut off and the liquor in the digester allowed to cool until the pressure in the digester had dropped to 60 pounds. The relief valve of the digester was then slowly opened, the digester opened, and the cage of chips was removed from the digester. The chips, after rinsing with cold water, were run through a kollar-gang with water, and were then run into a beater engine, in which the roll was raised a considerable distance above the bed. The pulp was beaten with water, gradually lowering the roll until at the end of the beating operating, which occupied about 60 minutes, the roll was about one-half turn up from the bed.

The beaten material was then run direct onto a screen and separated from the water, without any washing, and then the sheets were dried. This produced a pulp of rela-

tively great strength, a portion of which was repulped and made into paper, without any washing, other than by the water used in the pulping operation.

5 A sample of the paper so made, with a thickness of about .0073 inches, was tested and was found to have a breaking strength (Mullen test) of 80 pounds. Another sheet having a thickness of .0022 inches was found 10 to have a breaking strength of 20 pounds (Mullen test). Another sheet, having a thickness of 0.2 inch, had a Mullen test of 500 pounds. This is really a "plastic wood", as nothing whatever has been added, the 15 product being apparently the full contents of the wood with the exception of the sugars and other soluble constituents.

By the procedure above described it is possible to convert the raw wood into finished products and sheeted pulp in less than 20 three or four hours. Numerous tests which I have made indicate a yield substantially better than 90% based on the dry weight of the wood used.

25 The resulting paper in this example was of a yellowish or brownish color, somewhat darker than the ordinary manila stock, very well suited for wrapping paper on account of its high strength.

30 In other similar tests, blocks of wood, up to 150 cubic inches in size have been used in place of chips as above referred to, these being cooked about an hour or even an hour and a half, at 100 pounds pressure, with the 35 solution as above described.

#### Example 2.

White spruce was cut into chips averaging about three-fifths of a cubic inch in size. 40 These chips were digested in a solution containing about 1.4 ounces of sodium sulphate and about .3 ounces of copper sulphate per gallon. The cook was conducted at a pressure of about 85 pounds, at a temperature of 45 327° F. This high pressure was maintained only about 25 minutes, although the liquid was heated rather slowly, and after the source heat was shut off the cook was allowed to stand and cool simply by radiation 50 of heat from the digester until the pressure had fallen to about 45 pounds, when the relief valve on the digester was slowly opened. The chips, after soaking in water for a short time, were run, with water, through an ordinary pulper, then the resulting pulp was run 55 through the beater in the manner above indicated, for 45 minutes. At the commencement of this time the roll was raised five turns up from the bed and by lowering the 60 roll, a little at a time, at the end of the period the roll was about one-half a turn above the bed. The material was then divided into portions. One portion was sheeted into the form of molding pulp, producing 65 a light yellow-brown pulp. A sheet of

the pulp so produced, having a thickness of about .0045 inch was shown to have a strength of 60 pounds. The "plastic wood" in the form of articles molded under moderate pressure, was found to have great structural strength.

Another portion of the material, after a light washing, was made into paper, producing a very strong and relatively light colored paper of good strength and appearance. A sheet of this paper having a thickness of .007 inch was tested and found to have a strength of 80 pounds (Mullen test). A sheet .003 inch thick tested 48 pounds and a sheet .004 inch thick tested 55 pounds.

In this example, the period of time, when the temperature of the liquor in the digester was above 212° F., was considered as the cooking period, and this amounted to about 2 hours.

#### Example 3.

Hickory wood was digested in a solution containing about 1 ounce each of iron sulphate and sodium sulfate per gallon of liquor. The pulp was of a dark brown color and was very tough and strong. A sheet having a thickness of .005 inches, showed a strength of 55 pounds. The entire operation, from the raw wood to the sheeted pulp, occupied approximately 3 hours.

#### Example 4.

Oregon fir was treated with a solution containing about one and one-half ounces of potassium sulphate, per gallon of liquor. The sheeted material had a grayish color and was moderately strong.

#### Example 5.

Marsh growth, largely sedges, was digested in a 1.5% solution of magnesium sulfate, and run through the beater. This was then, without washing, made into paper of about the thickness of ordinary wrapping paper. 110 The product was very strong, tough and flexible. The pressure in the cooking was around 30 pounds, and the total cooking time (temperature over 210° F.,) was about an hour.

#### Example 6.

The stalks of hop vines were digested in a solution containing 1% of magnesium sulphate and .6% of sodium sulfate, as in the previous example. A good quality of pulp was produced.

#### Example 7.

White maple was treated by the process of Example 2 and gave a golden brown paper of good strength and good appearance. The digestive solution contained one ounce of sodium sulfate and one ounce of zinc sulfate, per gallon.

Other woods, which have been used with

good results are the following, red maple, oaks, holly, sycamore, dogwood, long leaf pine, short leaf pine, old field pine, gum, hickory, beech and birch.

5 In addition to woods such as above referred to, the process is applicable to various other kinds of vegetable growths such as grasses, straw, bamboo and canes (*Machrospelta arundaria* and *M. tecta*) marsh 10 growths, including sedges and various stalks with or without leaves.

With grasses, sedges, straw, vines, and the like, a temperature not over 280° F., and a pressure between 35 and 40 pounds give excellent results.

With the cane and bamboo, the pressures and times may be about the same as for the woods.

The process has given extremely good results with mixtures of cane and wood.

*Example 8.*

A mixture of green cane (70 parts) and green pine wood (30 parts) was cooked with 25 a solution of 1½ ounces of sodium sulfate and 1½ ounces of potassium sulfate per gallon. The cane, before cooking, was cut into lengths of about a foot, and the pine was cut into chips of average size of about 30 2 cubic inches. About 2½ pounds of the cane and wood were used, per gallon of liquor. The liquor was hot when the cane and wood were introduced. The material in the digester was heated to 100 pounds pressure, in 35 about 50 minutes; this pressure was maintained for an hour, and the heat then shut off, allowing to cool to about 5 pounds pressure in 75 minutes, the liquor blown out and the cooked material removed and thrown 40 into cold water overnight. The material was then run through a pulper of the mill-feed type, with water, then was beaten for an hour in a standard beater. A part of this was sheeted forming an extremely strong 45 carton stock, of a rather light tan color. This material was shown to be excellent for shoe counters etc., being about double the strength of the best high grade board stock on the market. High grade board (the best 50 grade found by me on the market) of a thickness of .035 inch, tested 190 pounds, while a product made by the present example, from green cane and green short leafed pine, of the same thickness tested 55 385 pounds. Another sheet of this latter material, .01 inch thick, tested 195 pounds.

In another case, I digested green cane material (3 parts) with  $\text{Na}_2\text{SO}_4$  solution (3%) and mixed this with green pitch pine (about 60 1 part) digested in  $\text{CuSO}_4$  solution (2%) giving a very strong material for carton stock, shoe counters, etc. In other cases 65% of green cane stock digested with  $\text{K}_2\text{SO}_4$  solution was mixed with green gum stock 65 digested with  $\text{Na}_2\text{SO}_4$ ,  $\text{CuSO}_4$ ,  $\text{FeSO}_4$ , or

mixtures of these. In such mixtures 65 to 75% of the cane material was used with 25 to 35% of the wood material. I also find that good results can be secured by mixing cane pulp with wood pulp, the latter being 70 made by the soda process, sulfite process or the old so called "sulfate process".

I call attention also to the fact that in the treatment of wood chips, it is possible to add from ten to twenty per cent or so of saw 75 dust or any other wood waste in the digester whereby the cost of the finished pulp can be materially lowered.

There appears to be a substantial advantage of using woods, cane, grasses, marsh 80 growths, etc., in the green state, rather than wholly dried, in that stronger products are generally produced. The complete drying of the material, before cooking, seems to weaken the fibers, to some extent at least. 85 Plant growths in either the green or dried condition can be readily reduced by my process.

As the result of my researches, the magnesium sulfate, alone or with alkali metal sulfate, as well as solutions of zinc sulfate with alkali metal sulfate, appear to give better results with grasses, bamboo, etc., than with resinous woods. Both of these give good 90 results with the non-resinous woods. 95

Sodium sulfate alone, or mixed with metallic sulfates seems to give better results with fir, spruce and hardwoods. Potassium sulfate alone or mixed with metallic sulfates seems to give better results with grasses, straw, bamboo, various stalks and marsh growths. These latter are apparently better treated with magnesium sulfate or with this plus an alkali metal sulfate. Aluminum sulfate alone or mixed with alkali metal sulfates reduces all plant growths well, but particularly with some of the woods, seems to harden the fibers to some extent. Tests also have shown that chromium sulfate gives somewhat darker colors to wood fibers and this material also colors some of the individual fibers from other growths as herein mentioned. Mild solutions of chromium sulfate give less darkening than strong solutions thereof (within the range of strengths 100 herein referred to). 110 115

In digesting wood, there is sometimes an advantage in using sodium sulfate alone, rather than potassium sulfate, magnesium sulfate or mixtures, in that in cooking with 120 sodium sulfate (especially during the first four or five cooks with such solution) a somewhat lighter colored pulp is produced and the fibers mat and weave well.

With any or all of these reagents, the bark 125 can be removed from the logs, slabs, etc., before cooking, if desired, or the bark can be left on the wood, if desired.

In the digestion, when treating woods, cane, etc., it is preferable not to exceed a 130

temperature of 337° F., with a pressure of 100 pounds, and it seems to be best not to exceed a temperature of 320° F., with a pressure of 85 pounds. With grasses, particularly, very favorable results are produced when the temperature does not exceed 280° F., with a pressure not over 35 pounds.

With woods, pressures not over 140 and best not over 125 pounds, are preferred.

- 10 When magnesium sulfate is to be used as the largest saline constituent of the digestive solution, it is advisable when digesting cane, grasses, marsh growths, etc., to use some  $K_2SO_4$  with this (say an amount equal to at least 8%, and preferably up to 12%, of the weight of the  $MgSO_4$ ). This tends to keep the silica in suspension. With woods, and especially the resinous woods, it is advisable to add about this proportion of sodium sulfate. In the case of the cane, grasses, etc., the material works freer on the screens, especially if the digestive solution has already been used in several successive cooks. This prevents the formation of gelatinous silica which would clog the screens.

*Example 9.*

The following example is given of Epsom salt ( $MgSO_4 \cdot 5 H_2O$ ), alone as the digestive solution.

Green pitch pine in the form of blocks 3 inches long, 1 inch wide and  $8\frac{1}{2}$  inches wide were filled into the digester in a basket or cage, and a cold solution containing 2% of the crystallized salt run in. The cook was heated until a pressure of 100 pounds showed in the digester, (requiring about 105 minutes heating). This pressure was held for 45 minutes and the contents then allowed to cool to about atmospheric pressure. The blocks were then run through a roller mill, then with water run through a pulper, and heated an hour. The yield was about 82%. This gave a strong pulp.

While I usually prefer to employ some  $Na_2SO_4$  or  $K_2SO_4$  with the  $MgSO_4$ , satisfactory results can be secured with the latter alone, especially when it is not desired to use the same cooking liquor for more than two or three cooks.

In most of the work done thus far, I have used fresh water in which to dissolve the sulfates. However, I note that salt water, (e. g., sea water) can be used if desired, and this is of advantage in the case of mills located on the salt water. It is noted that in Example 1, 7 gallons of the sodium sulphate liquor, containing about 1.8 ounces of sodium sulphate per gallon, to 10 lbs. of wood, will correspond to about .78 lbs. of the sulphate for each 10 lbs. of wood, or the amount of chemical is about 7.8%, based on the amount of wood.

Likewise in Example 2, the proportions given (assuming the same ratio of wood to

liquor) would correspond to about 7.3% of chemical, on the amount of wood.

In Example 8, a somewhat stronger solution was used, but a smaller amount thereof. Thus a gallon of liquor containing 3 ounces of salts,  $2\frac{1}{2}$  lbs. of cane and wood will correspond to about 7.5% of chemical relative to the wood, cane, etc.

The strength of solutions, as above given, are those which have been found to give excellent results. The solutions can be somewhat weaker, or stronger, without departing from the invention. For most purposes it is advisable not to employ less than half an ounce per gallon nor substantially more than four ounces per gallon. Stronger solutions are wasteful, and in some instances might considerably injure the product.

The expression "soluble sulfate of a metal having an atomic weight between 23 and 39.1" as used herein, is intended to embrace the sulfates of sodium, magnesium, aluminum and potassium, hereinabove mentioned, as well as mixtures containing one or more of these.

I claim:

1. In the manufacture of pulp from cellulosic and ligneous material, the improvement which comprises digesting such material with a solution of an alkali metal sulfate, substantially free from sulfid and substantially free from mineral acids.

2. In the manufacture of pulp from cellulosic and ligneous material, the improvement which comprises digesting such material with a solution of an alkali metal sulfate together with another sulfate such solution being substantially free from caustic alkali.

3. In the manufacture of pulp from cellulosic and ligneous material, the improvement which comprises digesting such material with a solution containing an alkali metal sulfate, as substantially its only dissolved active material, such solution containing one-half to five ounces of sulfate per gallon of liquor.

4. A process which comprises cooking mixtures of wood material and cane material, and sawdust and similar wood waste, in a hot digestive fluid containing an alkali-forming metal sulfate as its principal active dissolved material, such solution being free from free caustic alkali and from sulfids and from sulfurous acid, and being of a strength below 4%.

5. A process of making pulp which comprises digesting in a cooking liquor containing not substantially over 4% of a sulfate, a mixture of chips with up to 20% of sawdust and other small wood waste, such solution being free from substantial amounts of free mineral acid.

6. In the treatment of cellulosic material, the step of digesting the same with a solu-

tion containing a readily soluble sulfate of an alkali-forming metal, of substantially below 4% strength, such solution being free from substantial amounts of free mineral acid.

7. In the treatment of cellulosic and ligneous material, the step of digesting the same with a solution containing a readily soluble sulfate of an alkali-forming metal, 10 in amount corresponding to about 1 to 4 ounces per gallon of liquor, such solution being free from substantial amounts of free mineral acid.

8. In the treatment of cellulosic and ligneous material, the step of digesting the same with a solution containing magnesium sulfate and a sulfate of an alkali metal.

9. A process which comprises cooking mixtures of wood material and cane material, in a digestive fluid.

10. A process which comprises cooking green cellulosic and ligneous material in a solution of an alkali-forming metal sulfate of 1 to 4% strength.

11. A process which comprises digesting cellulosic and ligneous material, while hot and under pressure, with a solution containing a soluble sulfate of a metal having an atomic weight between 23 and 39.1, such 25 solution being substantially free from caustic alkali, free from alkali-metal sulfids, and free from sulfurous acid.

12. The herein described process which comprises subjecting a cellulosic material to 35 a cooking treatment by digesting the same in a solution, under superatmospheric pressure, and at near the boiling point of the solution for the existing pressure, such solution containing a readily soluble alkali-forming metal sulfate as its principal dissolved active component, but such solution being free from substantial quantities of sulfid, sulfite and hydroxid, until the intercellular cementitious matter in such cellulosic material is rendered friable throughout the pieces of such material, whereby the said pieces, although retaining their original form, become capable of being readily crushed, and thereafter reducing the material to a pulp.

13. The herein described process which comprises subjecting pieces of wood of any kind to a cooking treatment by digesting the same in a solution at a temperature at 55 which such solution boils under the existing pressure, said solution containing a sulfate of a metal having an atomic weight between 23 and 39.1, such solution being free from substantial amounts of sulfurous acid, until the cementitious matter in such cellulosic material is rendered readily friable throughout the pieces of such material, and stopping the digestion while the said pieces still retain their original form, but have become

capable of being readily crushed, and thereafter reducing the material to a pulp.

14. The herein described process which comprises subjecting a cellulosic material to a cooking treatment by digesting the same in a hot solution containing a sulfate of a metal having an atomic weight between 23 and 39.1, such solution being free from substantial amounts of sulfurous acid, until the cementitious matter in such cellulosic material is rendered readily friable throughout the pieces of such material, and until the said pieces, although retaining their original form, become capable of being readily crushed, and thereafter mashing the pieces of such material.

15. The herein described process which comprises subjecting a cellulosic material to a cooking treatment by digesting the same in a hot solution containing a sulfate of a metal having an atomic weight between 23 and 39.1, such solution being free from substantial amounts of sulfurous acid, until the cementitious matter in such cellulosic material is rendered readily friable throughout the pieces of such material, and until the said pieces, although retaining their original form, become capable of being readily crushed, soaking the cooked material in water and thereafter mashing the same.

16. A process which comprises digesting cellulosic and ligneous material in the form of pieces much larger than the commonly used wood chips, in a solution containing a metal sulfate, which solution is of a strength not substantially above 3%, which solution is substantially free from zinc salts, caustic alkali, soluble sulfides and sulfurous acid, continuing such digestion until the intercellular cementitious material is rendered readily friable, but not until the said pieces of material are substantially broken up or reduced to a pulp, and thereafter crushing such digested material while wet, without grinding the same, and thereafter reducing the crushed material with water to a pulp.

17. A process which comprises digesting wood in the form of pieces much larger than the commonly used wood chips, in a solution containing a soluble sulfate of an alkali-forming metal sulfate, which solution is of a strength not substantially above 3%, and being substantially free from zinc salts, caustic alkali, soluble sulfides and sulfurous acid, continuing such digestion until the intercellular cementitious material is rendered readily friable, but not until the said pieces of wood are substantially broken up or reduced to a pulp, and thereafter crushing such digested wood while wet, without grinding the same, and thereafter reducing the crushed wood with water to a pulp.

18. A process which comprises digesting woody material in a solution containing a

dissolved sulfate of a metal selected from the  
herein described group consisting of sodium,  
magnesium, potassium, copper, iron, cobalt,  
nickel, manganese and chromium, such solu-  
5 tion being of a concentration substantially  
below 4%, such solution being free from sul-  
furous acid, bisulfites, caustic alkali and  
soluble sulfides, until the intercellular cem-

10  
entitious matter is rendered friable but  
stopping the digestion while the pieces of  
woody material still have substantially their  
original size and shape, and thereafter crush-  
ing the digested material while still wet, and  
reducing it to a pulp.

In testimony whereof I affix my signature.  
ROBERT A. MARR.